

## UNITED STATES PATENT OFFICE

1,989,802

## SYNTHETIC TANNING MATERIAL

William F. Hester, Drexel Hill, Harry R. Raterink,  
Philadelphia, and Ian C. Somerville, Fox Chase,  
Pa., assignors to Rohm & Haas Company, Phil-  
adelphia, Pa.

No Drawing. Application October 10, 1932,  
Serial No. 637,100

13 Claims. (Cl. 260—3)

This invention relates to new synthetic tanning materials.

It is well known that sulphonic acids of aromatic hydrocarbons may be condensed by means of 5 aldehydes to produce substances which will precipitate gelatin, and convert hides or skins into leather. Similar products may be secured by condensing aromatic hydrocarbons first with aldehydes, and rendering the resinous materials 10 so obtained water soluble by sulphonation. These reactions have been carried out starting with many varieties of organic compounds, such as naphthalene, tetrahydronaphthalene, anthracene, phenanthrene, carbazole, phenol, cresol, 15 naphthol, while various aldehydes have also been employed, such as formaldehyde, acetaldehyde, furfuraldehyde, benzaldehyde. As a modification of these two types of reaction it has also been proposed to condense a sulphonated aromatic hydrocarbon with a nonsulphonated nucleus by means 20 of an aldehyde. For example in U. S. Patent #1,278,229 naphthalene sulphonic acid is condensed with an insoluble naphthalene hydrocarbon by means of formaldehyde. In this way an increased combining weight of the tanning material is secured, giving a product in many cases 25 intermediate in tanning properties between those made by condensing a sulphonated hydrocarbon and sulphonating a condensed hydrocarbon.

By an extension of this type of reaction to a large number of materials we have now discovered that by suitable selection of the unsulphonated material new products may be secured which have quite outstanding tanning properties. Of the 30 materials tried we have found that salicylic acid is by far the best for use in this connection, though others such as parahydroxybenzoic acid, parachlorophenol, and the like give good, though not surprisingly good results.

We are aware that salicylic acid has been utilized previously in the preparation of tanning materials. For example in U. S. Patent #1,344,950 a process is described for sulphonating salicylic acid and condensing by means of 35 formaldehyde. Further in German Patent #512,405 it has been proposed to condense salicylic acid with formaldehyde in an alkaline medium then to acidify and condense with resorcinol. It has also been suggested in condensations 40 where urea is used in conjunction with phenol sulfonic acid and formaldehyde, that hydroxy-carboxylic acids be also incorporated in the mixture, German Patent #539,474.

We now find however that by the addition of 45 relatively small amounts of salicylic acid to aro-

matic sulphonic acids in a medium of sulphuric acid of non-sulphonating strength, the subsequent formaldehyde condensation proceeds very smoothly in the absence of any nitrogenous material, to yield products whose tanning properties are far superior to those made by corresponding reactions without salicylic acid present.

The invention is illustrated in the examples below which are representative of various types of materials which can be used in this reaction. 10 It is obvious however that other extensions will readily suggest themselves to one skilled in the art, and the invention is not confined to the examples given. Of course, the method of sulphonation of the aromatic hydrocarbon is immaterial since it makes no difference in applicants' process whether sulphuric acid or some other sulphonation agent has been used such as oleum or chlorosulphonic acid, etc.

Example 1

128 grams of naphthalene is heated at 130° C. with 128 grams of sulphuric acid (98%) until water soluble. The temperature is dropped and 25 75 cc. water added, then 48 grams salicylic acid, and the temperature adjusted to 85° C. while 73 grams formaldehyde (37%) is run in slowly. Temperature is raised to 100° C. and maintained at this point until satisfactory condensation is 30 achieved. The mixture is diluted and the excess of mineral acid neutralized by soda ash. This solution may be used directly in tanning.

Example 2

54 grams of p-cresol is heated with 75 grams 35 of sulphuric acid (98%) for one hour at 75° C. To this is added 36 cc. of water, 13.8 grams of salicylic acid and 40 grams of formaldehyde (37%). The condensation mixture is heated at 75° C. for 2½ hours. Then the product is diluted 40 and treated with enough alkali to neutralize the excess mineral acid. The solution may be used directly for tanning.

Example 3

50 grams of crystalline paratertiary amyl- 45 phenol is heated with 47.5 grams of sulphuric acid (66° Bé.) for two hours at 90—95° C. To this is slowly added 22 cc. of water, 8 grams of salicylic acid and 25 grams of formaldehyde (37—8%). The condensation is continued for four hours at 50 85° C. The brown, viscous product is diluted and treated with enough alkali to remove the excess mineral acid. The solution may be used directly for tanning.

*Example 4*

51.5 grams of diisobutylphenol is heated with 38 grams of sulphuric acid (98%) for one hour at 75° C. To this is added 18 cc. of water, 6.9 grams of salicylic acid and 20 grams of formaldehyde (37%). The product is heated at 85° C. for four hours and then finished as in the preceding examples.

10

*Example 5*

228 grams of 4-4'-dihydroxydiphenyldimethylmethane is heated with 300 grams sulphuric acid (98%) at 65-70° C. for four hours, or until water solubility is obtained. 250 cc. water is now added, then 69 grams salicylic acid and temperature held at 50-55° C. while 97 grams of formaldehyde (37%) is run in. Heating is continued for five hours at 60-65° C., then the mixture diluted and the excess of mineral acid neutralized by addition of alkali. This solution may be used directly in tanning.

*Example 6*

66 grams of tetralin is heated with 75 grams of 98% sulphuric acid for 2 hours at 95° C. To this is added 38 cc. of water, 13.8 grams of salicylic acid and 40 grams of formaldehyde. The condensation and final preparation of the solution is similar to that in the preceding examples. A small amount of insoluble material which forms is removed by treating with charcoal and filtering. The filtrate may be used directly in tanning.

35

*Example 7*

56 grams of carbazole is heated with 100 grams of 98% sulphuric acid for 1 hour at 92° C. To this is added 48 cc. of water, 9.2 grams of salicylic acid, and 27 grams of 37% formaldehyde. The condensation and subsequent treatment is the same as given in Example 3.

*Example 8*

48 grams of  $\beta$ -naphthol is sulphonated with 50 grams of 98% sulphuric acid for 1 hour at 75° C. To this is added 24 cc. of water, 9.2 grams of salicylic acid and 27 grams of formaldehyde. The method of condensation and subsequent processing is the same as in Example 2.

*Example 9*

85 grams of o-phenylphenol is heated with 75 grams of 98% sulphuric acid for 1 hour at 75° C. To this is added 36 cc. of water, 13.8 grams of salicylic acid, and 40 grams of 37% formaldehyde. The rest of the procedure is the same as in Example 2.

60

*Example 10*

47 grams of phenol is heated with 74 grams of 98% sulphuric acid for 1 hour at 95° C. To this is added 36 cc. of water, 13.8 grams of salicylic acid, and 22 grams of acetaldehyde. The condensation is carried out for 2½ hours at 85° C. The subsequent treatment is the same as for Example 3.

70

*Example 11*

47 grams of phenol is sulphonated as in the preceding example. To this is added 36 cc. of water, 13.8 grams of salicylic acid and 36 grams of n-butyraldehyde. The condensation conditions are the same as in the preceding example.

*Example 12*

47 grams of phenol is sulphonated as in Example 10. To this is added 36 cc. of water, 13.8 grams of salicylic acid and 53 grams of benzaldehyde. The condensation conditions are the same as in Example #10. The solution obtained may be used directly in tanning.

While these represent the preferred method of working, it is also possible in some cases to carry out the reaction by first condensing the aromatic sulphonate with formaldehyde, then adding salicylic acid and more formaldehyde and condensing till a water soluble product is obtained.

As an example 128 grams naphthalene is taken and heated at 130° C. with 128 grams sulphuric acid 100% until water soluble. The mixture is cooled, diluted with 80 grams water then 60 grams of aqueous formaldehyde 37% solution added. Heating is continued at 90° C. until condensation is complete. The mixture is diluted to 426 grams, then 55 grams salicylic acid added, and 40 grams more formaldehyde 37% solution. Heating is continued at 90° C. until the mixture is water soluble, then it is diluted, and the excess of mineral acid neutralized. The solution may be used directly in tanning.

The amounts of the reactants may be varied to a considerable extent, though in each case there is a range of conditions which will give the best results. For instance in Example 1, for 1 mol. of naphthalene sulphonic acid from 0.2 to 0.4 mol. of salicylic acid, and from 0.7 to 0.9 mol. of formaldehyde were found to give the most satisfactory results. Again in Examples 2, 3, and 4 for 1 mol. of sulphonated alkyl substituted phenol, the best amounts of salicylic acid were found to be from 0.1 and 0.5 mol., and of formaldehyde from 0.7 to 1.4 mols. In Example 5, for 1 mol. of sulphonated 4-4'-dihydroxy diphenyl dimethylmethane, it was found best to use from 0.1 and 0.5 mol. of salicylic acid and from 0.7 to 1.4 mols of formaldehyde. A similar optimum range exists for the other examples.

These materials find extensive use in tanning by the customary methods. For instance they can be used by themselves to convert pickled skins into good light-colored leather. Further in conjunction with vegetable tanning materials, they can be applied to the leather as a pretannage giving a mellow grain, or may be mixed with the vegetable tannins and applied as a blend tannage, or they may be used to bleach and improve the feel of completely tanned vegetable leather. Another method is to use them as a supplementary tannage for skins treated with aldehydes, when full leather of very light color is secured. Finally in conjunction with chrome tannage they serve as filling agents, giving mellow leather of very light color, particularly when used towards the end of or at the conclusion of a regular chrome tannage.

The actual details of applications in these tannages will readily suggest themselves to one skilled in the art.

It is understood that deviations from the above are possible without departing from the spirit of the invention, the scope of which is to be limited only by the following claims. No modifications claimed to the exclusion of others.

We claim:

1. Water soluble synthetic resinous tanning material consisting of a condensation product of an aldehyde, an aromatic sulphonate acid and one

5

10

15

20

25

30

35

40

45

50

55

60

65

70

75

- of the group consisting of salicylic, parahydroxybenzoic acids and parachlorophenol.
2. Water soluble synthetic resinous tanning material consisting of a condensation product of an aldehyde, an aromatic sulphonic acid and salicylic acid.
3. Water soluble synthetic resinous tanning material consisting of a condensation product of an aldehyde, a hydroxy aromatic sulphonic acid and salicylic acid.
4. Water soluble synthetic resinous tanning material consisting of a condensation product of formaldehyde, an aromatic sulphonic acid and salicylic acid.
5. Water soluble synthetic resinous tanning material consisting of a condensation product of formaldehyde, a hydroxy aromatic sulphonic acid and salicylic acid.
6. Water soluble synthetic resinous tanning material consisting of a condensation product of formaldehyde, a naphthalene sulphonic acid and salicylic acid.
7. Water soluble synthetic resinous tanning material consisting of a condensation product of formaldehyde, sulphonated alkyl-substituted phenols and salicylic acid.
8. Water soluble synthetic resinous tanning material consisting of a condensation product of formaldehyde, a tertiary amyl phenol sulphonic acid and salicylic acid.
9. Water soluble synthetic resinous tanning material consisting of a condensation product of formaldehyde, a diphenyldimethyl methane disulphonic acid and salicylic acid.

10. Water soluble synthetic resinous tanning material consisting of a condensation product of formaldehyde, a naphthalene sulphonic acid and salicylic acid, where the reactants have the molecular ratio—for 1 mol. of naphthalene sulphonic acid, from 0.2-0.4 mol. salicylic acid and 0.7-0.9 mol. formaldehyde.

11. Water soluble synthetic resinous tanning material consisting of a condensation product of formaldehyde, a sulphonated alkyl-substituted phenol and salicylic acid, where the reactants have the molecular ratio—for 1 mol. of sulphonated alkyl-substituted phenol, from 0.1-0.5 mol. salicylic acid and 0.7-1.4 mols formaldehyde.

12. Water soluble synthetic resinous tanning material consisting of a condensation product of formaldehyde, a tertiary amyl phenol sulphonic acid and salicylic acid, where the reactants have the molecular ratio—for 1 mol. of tertiary amyl phenol sulphonic acid, from 0.1-0.5 mol. salicylic acid, and 0.7-1.4 mols formaldehyde.

13. Water soluble synthetic resinous tanning material consisting of a condensation product of formaldehyde, a sulphonated alkyl-substituted phenol and salicylic acid, where the reactants have the molecular ratio—for 1 mol. of sulphonated 4-4'-dihydroxy diphenyl dimethylmethane, 0.1-0.5 mol. salicylic acid and 0.7-1.4 mols formaldehyde.

WILLIAM F. HESTER. 30  
HARRY R. RATERINK.  
IAN C. SOMERVILLE.